

May 20, 1969

E. POLACCO ET AL

3,444,682

TOW TREATMENT FOR PREPARATION OF HIGH-BULK YARNS

Filed Aug. 9, 1966



FIG. 1.



FIG. 2.



FIG. 3.



FIG. 4.

INVENTORS  
EZIO POLACCO  
FRANCESCO DENTI

BY

*Stevens, Davis, Miller & Mroden*  
ATTORNEYS

## 1

3,444,682

### TOW TREATMENT FOR PREPARATION OF HIGH-BULK YARNS

Ezio Polacco and Francesco Denti, Mestre, Italy, assignors to ACSA—Applicazioni Chimiche S.p.A., Milan, Italy

Filed Aug. 9, 1966, Ser. No. 571,299

Claims priority, application Italy, Aug. 10, 1965,

18,198/65

Int. Cl. D02g 3/02; D01d 5/20

U.S. Cl. 57—140

10 Claims 10

### ABSTRACT OF THE DISCLOSURE

A wholly oriented staple fiber of a polymer of acrylonitrile comprised of sharply defined alternate segments B and A along its longitudinal axis, said segment B being of reduced denier with respect to segment A by reason of its having been stretched to a length of about 1.1 to 2 times as great as that of the said segment A. Also, staple fibers of the aforesaid type after having been shrunk in tensionless condition and yarns and fabrics comprised of such staple. Further, processes for the preparation of such staple predicated upon heat plasticizing a tow of oriented and relaxed filaments in repeating spaced segments, then stretching said tow, cutting the same into staple and, where appropriate, shrinking the same.

This invention relates to a process for the treatment 30 of two for the preparation of novel high-bulk acrylic yarns.

More particularly, this invention relates to the preparation of high-bulk yarns comprising acrylonitrile polymers which possess uniform dyeing characteristics 35 and texture.

High bulk acrylic yarns are known in the art to provide fabrics having enhanced apparent value and cover. They are commonly provided by blending fibers having different physical characteristics such as shrinking and filament configuration, whether mechanically or self-induced. In the latter case bifilar or bicomponent fibers wherein the two components shrink differently to thereby cause crimp formation can be blended with monocomponent fibers to provide yarns from which fabrics, including carpets, having excellent cover and apparent value can be manufactured. While this technique is widely employed and provides excellent products, economics and processing difficulties demand other methods for producing high bulk yarns.

Thus, an alternate means for preparation of high bulk yarns lies in the blending of fibers which are different at least to the extent that they possess considerable variation in their ability to shrink upon treatment with heat. One known technique to achieve this type of blend lies in feeding separate tows having differing heat shrinkage properties to a staple cutter to thereby achieve a staple fiber blend in the desired proportion. One salient difficulty with such a blend lies in the observation that in subsequent textile processing operations, such as carding, combing and the like, the high shrinking fibers tend to migrate toward the core of the yarn thereby to create a yarn characterized, more or less, by a high shrinking core and even though such yarns develop bulk when subjected to heat treatment, they suffer losses of strength and aesthetic value.

More recently, attempts have been made to overcome the tendency for fibers to migrate in high bulk yarns as above indicated by the provision of yarns made from tow having continuously varying shrinkage properties along the longitudinal axis. Such a tow may have, for

## 2

example, from zero up to about 20 percent difference in shrinkage which varies along the length of the tow so that if the percent of shrinkage upon heat treatment were plotted against the length of the tow the plot would be sinusoidal. In practice, however, achievement of shrinkage differential large enough to provide good bulk characteristics in a yarn requires such a wide oscillation period that staple fibers prepared from such tows vary so greatly that the yarn tends to resemble a high-low shrinkage blend as above discussed.

It therefore becomes an object of the invention to provide a novel bulky acrylic yarn having uniformity, strength and high bulk.

Another object of the invention lies in the provision of a novel process for treatment of tow comprising filaments of acrylonitrile polymers to provide high-bulk yarns.

Additionally, this invention has as its object a novel staple fiber component of high-bulk yarns.

These and other objects of this invention are achieved by stretching a previously oriented and relaxed continuous tow comprised of filaments of acrylonitrile polymers having regularly intermittent heat plasticized segments along its length to provide a wholly oriented filamentary tow having repeating spaced segments of less than staple fiber length along the length of the tow which have been stretched to a greater degree than the remaining segments.

The tow having repeating spaced segments of fiber which have been stretched to a greater degree than the remaining segments may be prepared by continuously passing the tow over a heated roll having a channeled or tooth-like surface so that when the tow is passed over the roll only certain segments of the tow come into contact with the heated surface to thereby become plasticized. The tow having spaced plasticized segments is passed from the channeled roll in the plasticized condition to a set of draw rolls moving at a greater peripheral speed than the channeled roll thereby causing the partially plasticized tow to stretch in those segments which are in a heat plasticized state.

The tow obtained according to the process of this invention is characterized in that it is composed of individual filaments having regularly alternating stretched segments B which segments are heat shrinkable and segments A which receive no stretch according to the instant invention and which are not heat shrinkable or heat shrinkable only to a minor degree. The tow can then be cut to staple fiber of a desired length wherein each fiber component has high and low shrinkage segments along its longitudinal axis. Heat shrinkage of yarns prepared from these staple fibers creates a novel yarn which possesses uniform dyeing characteristics, high strength and high bulk.

The lengths of the high shrinking and low shrinking segments built into the tow (and the resulting ratio of B/A) must be chosen with consideration of characteristics desired in the final yarn such as bulk, fiber length, degree of heat shrinkage and the like. Preferably, the length of the high shrinking segments should be between about 15 and 100 millimeters. Similarly, the length of low shrinking segments should lie between about 15 and 100 millimeters. The choice of the lengths of the different segments should be such that the sum of A and B equals the cut length of the staple desired for conventional textile processing generally between about 80 and 120 millimeters.

The invention may be more clearly understood by reference to the accompanying drawing wherein;

FIGURE 1 represents a schematic of yarn treatment according to the instant process,

FIGURE 2 represents an illustration of a length of filament treated according to the instant process,

FIGURE 3 represents the length of filament shown in FIGURE 2 treated according to this process and having been subsequently heat shrunk and,

FIGURE 4 is a graph showing the stress-strain curves of yarn prepared according to this invention and an unbalked yarn.

More particularly, FIGURE 1 illustrates the process of this invention wherein a tow 1 of a previously uniformly stretched and relaxed acrylonitrile polymer fiber is continuously passed to feed rolls 2 and 3 and then to an idler roll 4 from whence the tow is passed on to the heated surface of channeled roll 5 which rotates (clockwise direction in FIGURE 1) at the same peripheral speed as feed rolls 2 and 3. Portions of the tow 1 contact heated roll 5 at heated teeth or contact elements represented by tooth or element 9 which may be an integral or permanent part of roll 5 or it may be attached as by screw, bolt or other means 10. Thus, segment A of tow 1 does not contact the surface of roll 5, while segment B of tow 1 contacts the heated surface of the roll as illustrated and is heated to the extent that it is plasticized. Upon leaving roll 5 tow 1 possessing continuously repeating A and B segments along its length is fed over idler roll 6 to draw rolls 7 and 8 which rolls rotate at a higher peripheral speed than rolls 2, 3, and 5 thereby causing the tow 1 to be stretched to a length of from about 1.1 to 2 times the length fed to rolls 2 and 3. Insofar as the repeating segments B leave roll 5 in a plasticized condition, all of the stretch applied to the tow occurs in these segments whereas segments A remain unmodified. As above indicated, channeled roll 5 presents a toothed surface to the tow wherein heat transfer is effected to the tow passing in contact with the heated surface of the teeth on roll 5. The several teeth may present uniform or different peripheral lengths of contact to the tow being passed over roll 5. Similarly, the peripheral lengths of the spacings between the several teeth may vary or be uniform. Moreover, their peripheral lengths may be the same as or differ from the peripheral lengths of the teeth. By suitably varying the profile of the channeled or toothed roll and the number of teeth or raised contact elements, it is possible to obtain a wide variety of combinations of stretch, stretch ratios, ratios between stretched and unstretched segments, and the like. Preferably, the outer surface of the raised contact elements have a rectangular shape although this is not a critical aspect of the invention so long as there is sufficient contact surface to transfer heat to the tow.

Roll 5 may be heated by electrical means, by high pressure steam, or by other suitable means for elevating the temperature of the teeth or raised contact elements to cause suitable softening or plasticizing of the filamentary material passing in contact therewith. The temperatures necessary to plasticize the filaments or tow lie between about 60° and about 200° C., more typically between about 90° and about 180° C.

Upon leaving draw rolls 7 and 8 the individual filaments of tow 1 may be characterized by segments along their lengths having sharply varying denier caused by differential stretching as depicted in FIGURE 2. Thus, A in FIGURE 2 represents that portion of the filament which is essentially unmodified by passing over roll 5 whereas adjacent segment B' has been heat plasticized and stretched to thereby cause some reduction in denier at sharply defined points along the length of the filament. Upon subjecting the filament depicted in FIGURE 2 to heat shrinkage the differences in denier disappear for all practical purposes and the filament represents a substantially uniform denier as depicted in FIGURE 3 having essentially uniform segment AB'A.

As above indicated this invention is applicable to yarns comprised of filaments of acrylonitrile polymers. These include polyacrylonitrile and interpolymers comprising

at least about 80 weight percent of acrylonitrile and up to about 15 percent of one or more monoethylenically unsaturated monomers interpolymerizable therewith. Comonomers such as methyl methacrylate, vinyl acetate, styrene, vinylidene chloride, vinyl bromide, vinylpyridine, alkenyl and alkenyloxysulfonic acids, and the like may be interpolymerized in minor amounts with acrylonitrile according to means well known in the art to form useful fiber forming polymers. The polymers of acrylonitrile, useful for this invention, may then be dissolved to form spinning solutions in dimethylsulfoxide, dimethylformamide, dimethylacetamide or the like and thereafter extruded by wet, dry, or dry jet-wet methods to form a multi-filament bundle of synthetic filaments which is coagulated, washed, stretched, dried and relaxed by any of several well known prior art processes. The tow treated according to this invention may be given a mechanical crimp after treatment on roll 5 to facilitate handling in subsequent textile operations such as combing and carding.

Moreover, roll 5 may be used to replace the heating plates in machines such as the Turbo-Stapler, the Seydel or Termatex converters and other machines employed to convert tow into top. The top thus obtained is comprised of individual fibers each having high and low shrinking segments along their longitudinal axes.

The following examples are given to illustrate the invention and should not be construed as defining the limits thereof insofar as variations incorporating the spirit of the invention hereinafter defined by the claims will be readily apparent to those skilled in the art. The bulk values reported were obtained using a Yarn Bulkometer by Linra.

#### Example I

A 40,000 filament tow of a polymer of 94 weight percent acrylonitrile and 6 weight percent vinyl acetate having a total denier of 120,000 having been stretched and relaxed was fed to a pair of feed rolls corresponding to roll 2 and 3 in FIGURE 1 and thereafter passed over a channeled roll corresponding to roll 5 heated to 130° C. and on to draw rolls 7 and 8. The peripheral speed of rolls 2 and 3 was 23 meters per minute while rolls 7 and 8 were run at a peripheral speed of 27.5 meters per minute to give the tow a 1.2× stretch. The hot channeled roll had an outer diameter of 300 millimeters with uniform raised contact surfaces of 30 millimeter spaced surfaces and channels spacing the raised contact surfaces of 55 millimeters, the ratio of heated contact periphery to spaces being 30/55. The tow thus treated was thereafter passed to staple cutter and cut to a length of 100 millimeters to provide individual staple fibers having both stretched and unstretched segments.

The staple fiber was then processed according to the worsted system to provide a yarn having the following properties:

|                   |             |
|-------------------|-------------|
| Metric count(nm.) | 34/2        |
| Twist             | 340 Z+220 S |
| Bulk              | 6-7         |

The yarn was then arranged in hanks, treated with boiling water in a dyeing cabinet and thereafter centrifuged and dried. The boiling water treatment caused the yarn to bulk uniformly to provide the following modified properties:

|                   |             |
|-------------------|-------------|
| Metric count(nm.) | 27/2        |
| Twist             | 420 Z+275 S |
| Bulk              | 18          |

Moreover, the yarn possesses a handle and appearance of woolen yarn and may be used for normal weaving as well as for hosiery.

The yarn was thereafter employed to manufacture a plain knitted fabric with a stitch length (L) of 5.6 millimeters and compactness (C) 20.6 where C=L mm. The

fabric so obtained was compared with a knitted fabric of the same compactness the fibers of which had not been treated according to the process of this invention. The novel fabric exhibited better stitch clarity and pilling (after 20 hours of Random Tumbler) of 12 mg./dm.<sup>2</sup> as compared with 14 mg./dm.<sup>2</sup> for the control fabric. Handle of the two fabrics was essentially equivalent.

*Example II*

The procedure of Example I was repeated using a 100,000 denier tow comprised of 20,000 filaments under the following condition:

|                      |                 |
|----------------------|-----------------|
| Stretch              | 1.15            |
| Length of B segment  | millimeters 25  |
| Length of A segment  | do 60           |
| Ratio B/A            | 25/60           |
| Channeled roll temp. | °C 100          |
| Staple length        | millimeters 100 |

The yarn obtained by the worsted processing cycle shows 20 the following characteristics:

|                    |             |
|--------------------|-------------|
| Metric count (nm.) | 34/2        |
| Twist              | 340 Z+220 S |
| Bulk               | 6-7         |

After heat treatment with steam the yarn characteristics 25 were:

|              |             |
|--------------|-------------|
| Metric count | 27/2        |
| Twist        | 420 Z+275 S |
| Bulk         | 19          |

The yarn produced by the procedure is similar in appearance and workability to woolen hosiery yarns. The characteristics of elongation and recovery are comparable to woolen yarns of equivalent bulk which renders the yarn quite suitable for hosiery products in contrast to acrylic high-bulk yarns obtained by previously known methods.

*Example III*

Repeating Example I with a 480,000 denier tow comprised of 60,000 filaments a novel yarn was prepared 40 under the following conditions:

|                      |                 |
|----------------------|-----------------|
| Stretch              | 1.5X            |
| Length of B segment  | millimeters 45  |
| Length of A segment  | do 40           |
| Ratio of B/A         | 45/40           |
| Channeled roll temp. | °C 180          |
| Length of staple     | millimeters 100 |

The yarn obtained was worked up according to the worsted wool cycle and showed the following characteristics before and after heat treatment by steam:

|                    | Before      | After       |
|--------------------|-------------|-------------|
| Metric count (nm.) | 34/2        | 26/2        |
| Twist              | 320 Z+220 S | 420 Z+275 S |
| Bulk               | 6-7         | 17          |

Elongation and recovery characteristics of the bulked 60 yarn were similar to those of woolen yarns of corresponding bulkiness.

*Example IV*

A 480,000 denier tow comprised of 160,000 acrylonitrile/vinyl acetate (94/6) filaments was processed on a Turbo-Stapler in which the heating plates had been replaced by a channel roll under the following conditions:

|                        |                  |
|------------------------|------------------|
| Feeding speed          | meters/minute 23 |
| Stretch                | 1.15X            |
| Roll temp.             | °C 160           |
| Stretch at break ratio | 3:20             |
| Nominal cut            | inches 6         |

The channeled roll used in place of the heating plates had a diameter of 300 millimeters, the contact lengths being 25 millimeters and the spaces being 60 millimeters.

Turbo-top thus obtained was processed on conventional textile machinery to provide yarn having a metric count (nm.) of 30/2, a twist of 310 Z+200 S and a bulk of 5-6. The yarn in hanks was shrunk in boiling water for about 30 minutes centrifuged and dried. The yarn resulting from shrinkage had the following properties:

|                    |             |
|--------------------|-------------|
| Metric count (nm.) | 23/2        |
| Twist              | 390 Z+250 S |
| Bulk               | 17          |

In comparison with bulked yarn obtained by conventional methods on a Turbo-Stapler, the yarn prepared as above described shows superior mechanical strength and exhibited a more uniform bulkiness. A plain knitted fabric having a stitch length of 5.6 millimeters and compactness of 10 was manufactured using the top above obtained and compared with a fabric manufactured from conventional top having the same compactness. The fabric of this invention showed superior stitch clarity and pilling of 4.8 as compared with 6.5 mg./dm.<sup>2</sup>. Handle was definitely softer than the control.

FIGURE 4 shows stress-strain curves wherein C represents yarn prepared according to this example and D represents yarn prepared from conventional Turbo-top. The break length is the length of yarn in kilometers required to break the yarn under its own weight. The curve plotted for the yarn prepared from tow treated according to the instant invention exhibits a more uniform development.

We claim:

1. Staple fibers, cut from a tow of wholly oriented filaments of a polymer of acrylonitrile having sharply defined alternate segments B of reduced denier along its longitudinal axis and said segments B being of less than staple fiber length and having been stretched to lengths about 1.1 to 2 times greater than the lengths of the remaining segments A of the tow, said remaining segments A also being of less than staple length, with the lengths of the respective segments being such that the sum of A and B equals the cut length of the staple.

2. A wholly oriented staple fiber of a polymer of acrylonitrile comprised of sharply defined alternate segments B and A along its longitudinal axis, said segment B being of reduced denier with respect to segment A by reason of its having been stretched to a length about 1.1 to 2 times as great as that of the said segment A.

3. Staple fibers according to claim 2 exhibiting substantially homogeneous cross-sections along their longitudinal axes by reason of their additionally having been shrunk in tensionless condition, whereby there were effected substantially uniform deniers thereof.

4. High-strength, high-bulk yarn susceptible to more uniform dyeing, comprised of the staple fibers of claim 3.

5. A fabric of the yarn of claim 4.

6. Yarn comprised of staple fibers according to claim 2.

7. A process for the preparation of wholly oriented staple fibers of a polymer of acrylonitrile individually comprised of sharply defined alternate segments B and A along their longitudinal axes, said segments B being of reduced diameter with respect to segments A by reason of their having been stretched to lengths about 1.1 to 2 times as great as that of the said segments A, comprising heat plasticizing a tow of oriented and relaxed filaments of a polymer of acrylonitrile in repeating spaced segments along the longitudinal axis of the tow, thereafter stretching said tow about 1.1 to 2 times while the heat plasticized repeating spaced segments thereof are still in a plasticized condition, and thence cutting the said tow into staple lengths of from between about 80 and 120 millimeters.

8. The process as defined by claim 7, further comprising shrinking said wholly oriented staple fibers in tensionless condition, whereby there are obtained staple fibers exhibiting substantially homogeneous cross-sections along their longitudinal axes.

9. The process as defined by claim 7, wherein the tow is heat plasticized in repeating spaced segments along its

longitudinal axis by passing said tow in longitudinal contact with repeating spaced heating elements situated on the periphery of a roll.

10. A process for the preparation of high-strength, high-bulk yarn susceptible to more uniform dyeing, comprising heat plasticizing a tow of oriented and relaxed filaments of a polymer of acrylonitrile in repeating spaced segments along the longitudinal axis of the tow, thereafter stretching said tow about 1.1 to 2 times while the heat plasticized repeating spaced segments thereof are still in a plasticized condition, and then cutting the said tow into staple length of from between 80 to 120 millimeters to form staple fibers, forming a yarn structure of said wholly oriented staple fibers and thence shrinking the same in tensionless condition whereby there are effected substantially uniform deniers thereof.

## References Cited

## UNITED STATES PATENTS

|           |         |                         |
|-----------|---------|-------------------------|
| 2,296,394 | 9/1942  | Meloon.                 |
| 2,917,779 | 12/1959 | Kurzke et al.           |
| 2,952,116 | 9/1960  | Burleson ----- 57—34 XR |
| 2,975,474 | 3/1961  | Smith.                  |
| 3,017,684 | 1/1962  | Pittman ----- 28—72     |
| 3,116,197 | 12/1963 | Kasey.                  |

10 STANLEY N. GILREATH, *Primary Examiner.*

15 W. H. SCHROEDER, *Assistant Examiner.*

U.S. Cl. X.R.

15 57—55.5, 157; 161—179; 264—167, 290